

## UNITED STATES PATENT OFFICE

2,116,843

## SHOT SHELL

John M. Olin, Alton, Ill., assignor to Western Cartridge Company, East Alton, Ill., a corporation of Delaware

No Drawing. Original application October 6, 1923, Serial No. 667,075. Divided and this application April 30, 1930, Serial No. 448,800

5 Claims. (Cl. 102—15)

The invention relates to a loaded cartridge and more particularly a cartridge in the nature of a loaded shot shell employing a double base powder such as nitrocellulose-nitroglycerin powder. This application is a division of application Serial Number 667,075, filed October 6, 1923, Patent No. 1,757,584, issued May 6, 1930.

The burning action of dense nitrocellulose powders is often accelerated by the addition of nitroglycerin. Such a powder, however, produces a propellant charge which will burn quickly and may be almost consumed at the initial stage. In a cartridge employing such a powder, the maximum pressure is not developed or sustained for any appreciable distance along the gun barrel, but the initial pressure drops rapidly to its minimum. Accordingly, the total energy utilized is practically that released upon the initial combustion of the charge. A shot shell employing such a powder is therefore limited as to its zone of energy transfer because of the limiting breech pressure.

One of the objects of this invention therefore is to provide a shot shell containing a shot-propelling charge of granular double base smokeless powder, and more particularly a nitrocellulose-nitroglycerin powder, which powder is in such form, so modified and so primed and so confined as to burn progressively when fired in a shot gun.

Further objects will appear from the detail description, in which will be described an illustrative embodiment of this invention; it will be understood, however, that this invention is not limited to the specific embodiment disclosed.

In accordance with this invention a shot shell comprising, a case or shell, a coordinative primer therein, a shot charge and wadding, has a shot-propelling charge of a double base powder which is made progressive burning by retardation of its initial combustion rate. This may be accomplished by modification of the grain, as by surface treating the grain with a deterrent and by proper priming and confining of the powder charge. An illustrative embodiment of this invention comprises a nitrocellulose-nitroglycerin powder grain surface treated with dinitro-toluene. The double base powder is surface-modified or treated in coordination with the primer to substantially retard its initial combustion rate and the accelerator in the interior of the grain is adapted in coordination with the retarder or deterrent to maintain a fast subsequent burning rate, as by making the nitroglycerin content such as to secure that result.

A double base powder of this character when loaded in a shot shell and when suitably primed and confined with reference to its surface and core, will cause the shot charge to be propelled at a reduced breech pressure as compared to nitrocellulose-nitroglycerin powders not so treated; moreover, the shot charge is started comparatively gradually, while the velocity imparted to the projectile charge is maintained with the acceleration more gradual than in nitrocellulose-nitroglycerin powders not so treated. Moreover, the pressure rises slowly to a comparatively flat peak and drops slowly, and this pressure is sustained for an extended distance along the gun barrel, all as compared to shot shells employing double base powders not so treated. These characteristics of a progressive burning double base powder when employed in a shot shell for propelling the shot charge, not only materially reduce the stringing of shot but also improve the pattern.

The propellant charge is properly coordinated with the other components of the shot shell, by coordination with the primer, the wadding and the shot charge. The primer, therefore, is preferably a comparatively hot primer so as to insure ignition of the surface treated grains as well as continuation of the burning of the powder charge, while the wadding is made sufficiently heavy to secure the desired confining of the powder charge in order to cause the pressure to be maintained, so as to insure the continuation of the burning of the powder.

In accordance with this invention, a double base powder, such as nitrocellulose-nitroglycerin powder designed for use in a shot shell, is treated so as to burn progressively. This can be accomplished by surface treating such a powder, containing the desired percentage of nitroglycerin and granulated or sub-divided to the desired or required granulation, such as thirty mesh in any suitable manner so as to render it progressive burning. A deterrent which is particularly suitable is dinitro-toluene, which can be applied in any manner, as by tumbling in a rotating drum at a temperature of about 80° C. for about one-half hour, using about 2% of the deterrent relative to the weight of the powder, so that the powder grains will become impregnated with the deterrent. It will be understood that the above is simply an illustrative embodiment; for the amount of the deterrent employed and the period of treatment, and to some extent even its temperature, as well as other conditions of treatment, will vary with and depend upon the char-

acter and composition of the powder grain, of the deterrent employed and the intended use of the powder, as well as the desired characteristics which this powder grain is to have. The object 5 is to subdivide the powder to an extent sufficient and to impregnate each powder grain of the desired composition to an extent sufficient and with sufficient of the deterrent to cause the powder when confined and primed, as previously described, to burn progressively when fired in a shot gun.

As a further illustrative embodiment of this invention, a progressive burning double base powder can be secured by incorporating with the 15 nitrocellulose and nitroglycerin where the percentage of nitroglycerin is high (35%-40%), and preferably during the course of manufacture, a cooling or slowing agent having the action of reducing the temperature of burning and slowing 20 up the combustion in such a manner as to produce the desired result followed by a surface treatment as described. There are many compounds which may be used for this purpose, among them being: vaseline and similar products, alkaline bi-carbonates, either alone or mixed with vaseline, diethyl diphenylurea, dimethyl diphenylurea, cyanamide, tartrates, olive oil, castor oil, fats and resins, soaps, oxalates, starch, dextrose, and diphenylamine. All of these are classed 25 as deterrents and they may be incorporated with the nitrocellulose base together with the nitroglycerin. Such nitrocellulose-nitroglycerin powders, containing from 35% to 40% of nitroglycerin, together with a cooling or slowing agent of 30 the character described, may be surface treated with dinitrotoluene as heretofore described. It will be understood that the above is simply illustrative of an embodiment of this invention; for the percentage of nitroglycerin and the character 35 of the slowing agents if employed will vary, of course, with the characteristics which the powder is to have, as well as the uses to which it may be put and the situations in which it may be employed. It will be understood in this connection 40 that nitroglycerin serves as a component of the core to sustain the combustion, and also to overcome to some extent the delayed ignition characteristics imparted by the surface treatment.

In accordance with this invention a shot shell 45 is produced in which the powder will burn progressively so as to develop its energy in such a manner that the energy released and imparted to the shot charge is very much greater for the same and limiting breech pressures than in shells 50 using other powders. In the shell embodying this invention, a given charge of shot (such as 1 1/4 oz. in a 12 gauge shell) can therefore be propelled a greater distance as compared to other shells; accordingly, a greater shot charge can be projected 55 the same distance as in other shells using other powder; and all at the same limiting and safe breech pressures. This means that the shell embodying this invention will operate in a zone of high energy transfer at safe breech pressures 60 because the powder will burn progressively in such a zone. The range and pattern is improved and shot stringing decreased.

While the invention is particularly applicable

to the type of cartridge specifically described, it will be understood that the invention is applicable as to many of its aspects to other forms and types of cartridges. It will further be understood that while dinitrotoluene has been specifically referred to as a deterrent, other suitable deterrents, having the desired properties and imparting to the powder of the desired composition the desired characteristics, may be employed. It will furthermore be understood that certain features 10 and sub-combinations are of utility and may be employed without reference to other features and sub-combinations; that is contemplated by and is within the scope of the appended claims. It is furthermore obvious that various changes may be 15 made in details, within the scope of the appended claims, without departing from the spirit of this invention. It is therefore to be understood that this invention is not to be limited to the specific details described.

Having thus described the invention, what is claimed is:

1. A loaded shot shell comprising a case or shell, a coordinative primer therein, a shot charge, wadding, and a shot-propelling charge of 25 granular double base smokeless powder which is surface-modified in coordination with the primer to substantially retard the initial combustion rate.

2. A loaded shot shell comprising a case or shell, a coordinative primer therein, a shot charge, wadding, and a shot-propelling charge of 30 granular nitrocellulose-nitroglycerin powder which is surface-treated with dinitrotoluene in coordination with the primer to substantially re- 35 tard the initial combustion rate.

3. A loaded shot shell comprising a case or shell, a coordinative primer therein, a shot charge, wadding, and a shot-propelling charge 40 of powder grains containing at their surfaces a retarder of combustion coordinated with the primer to substantially retard the initial combustion rate, said grains having in their interiors an accelerator of combustion adapted in coordination with the retarder to maintain a fast sub- 45 sequent burning rate.

4. A loaded shot shell comprising a case or shell, a coordinative primer therein, a shot charge, wadding, and a shot-propelling charge 50 of granular double base smokeless powder, viz. nitrocellulose-nitroglycerin powder, which is surface modified in coordination with the primer to substantially retard the initial combustion rate, the nitroglycerin content being such in coordination with the surface modification as to main- 55 tain a fast subsequent burning rate.

5. A loaded shot shell comprising a case or shell, a coordinative primer therein, a shot charge, wadding, and a shot-propelling charge 60 of smokeless powder grains composed of nitro- 65 cellulose containing nitroglycerin and a deterrent, said grains being surface-treated with a deterrent coordinated with the primer to sub-stantially retard the initial combustion rate, and the nitroglycerin content being such in coordi- 70 nation with the deterrent as to maintain a fast subsequent burning rate.

JOHN M. OLIN.